

## 1

3,672,977

### PRODUCTION OF POLYESTERS

Kimon Constantine Dardoufas, Richmond, Va., assignor to Allied Chemical Corporation, New York, N.Y.  
No Drawing. Filed Oct. 26, 1970, Ser. No. 84,168

Int. Cl. C08j 1/44; D06m 13/00

U.S. Cl. 117—138.8 F

1 Claim

### ABSTRACT OF THE DISCLOSURE

An improved multifilament polyethylene terephthalate yarn having a lubricating protective film applied thereon of from about 0.3 to about 0.6 weight percent based on the weight of the yarn of a liquid composition consisting essentially of about 10 to about 20 weight percent of said composition of each hexadecyl stearate and refined coconut oil, about 3.0 to about 6.0 weight percent of said composition of ethoxylated tallow amine, about 10 to about 20 weight percent of said composition of ethoxylated lauryl alcohol, about 8.0 to about 12.0 weight percent of said composition of sodium salt of alkylarylsulfonate, about 1.0 to about 3.0 weight percent of dinonyl-sodium-sulfosuccinate, about 1.0 to about 3.0 weight percent of said composition of 4,4'-thio-bis-(3-methyl-6-tert-butylphenol), about 35 to 50 weight percent of said composition of white mineral oil having a boiling point of between 510° F. and 620° F. wherein at least about 0.15 to about 0.30 weight percent is retained on said yarn, and then treating said yarn with from about 0.7 to about 1.2 weight percent on said yarn of a liquid composition selected from the group consisting of (a) about 95 to about 98 weight percent of said composition of triethylene glycol-dipelargonate and about 2 to about 5 weight percent of said composition of 2,2'-methylene-bis-(4-methyl-6-tert nonylphenol), and (b) about 13 to about 25 weight percent of said composition selected from the group consisting of glycerol monoleate and decaglycerol tetraoleate with ethoxylated tall oil fatty acids, about 12 to about 20 weight percent of said composition selected from the group consisting of sulfated glycerol trioleate and ethoxylated alkylamine, and about 55 to about 75 weight percent of said composition of hexadecyl (isocetyl) stearate.

### BACKGROUND OF THE INVENTION

This invention relates to improved multifilament yarns, and particularly to multifilament polyethylene terephthalate yarns for industrial uses. More particularly it relates to a new finishing process for polyester yarns in which novel finish compositions are applied to said yarns.

Synthetic continuous filament yarns are produced wherein lubricating compositions containing antistatic properties are applied in order to meet processing requirements and particularly at high speeds. As greater requirements are made on the physical properties of such yarns in light of new and improved safety regulations with respect to their ultimate end use, the compositions must contain materials, for example, as yarn to cord conversion efficiency, cord to rubber adhesion, improved fatigue properties, improved thermal stability, etc. In known prior practice of utilizing a one step finish, that is, a spin finish which would support an efficient fiber process performance while at the same time would provide the desired tire cord properties, a compromise must always be accepted between fiber process efficiency and tire yarn surface requirements.

Accordingly, it is an object of this invention to provide an improved polyester continuous filament yarn and an improved process for preparing said yarn. A further object of this invention is to provide an improved polyester filament yarn and an improved process for preparing

## 2

said yarn for reinforcing rubber tires, by using first, an improved composition for use as a process finish, followed by an improved composition for use as yarn to yield the desired yarn cord properties.

5 Polyester yarns are known to be drawn at elevated temperatures and thermal variability depends upon the thermodynamic properties of the finish which effects processing performance as well as yarn physical properties. Therefore, parameters such as low finish specific heat and, low heat of vaporization of the volatile components and the lowest finish level required for fiber protection are essential to minimize heat losses for good fiber processing performance. This illustrates the inferior performance of all aqueous finishes in comparison to the non-aqueous finishes which can be applied at a level significantly lower for the same or equivalent percent solids on yarn and have much lower specific heat and heat of vaporization compared to aqueous or water base material.

The improved composition for use as the process finish 20 in accordance with this invention consists of a non-aqueous homogeneous blend of lubricants; emulsifiers, antistat, wetting agent; and, an antioxidant. The blend is a clear liquid free of suspended solids, and having a viscosity of 27 centipoises at room temperature, a surface tension of 25 about 32 dynes per centimeter and a contact angle on polyester of about 9°, which insures proper wetting ability for uniform distribution of the composition. The lubricating and continuous phase of the composition consists of about 39 weight percent mineral oil of low viscosity of 30 about 40 SSU at 100° F., flash point of 260° F., and boiling range of about 510° F. to 620° F., about 14.5 weight percent coconut oil and 14.5 weight percent hexadecyl stearate which have low volatility and excellent heat stability. The remainder consists of about 10 weight percent 35 of natural petroleum sulfonate (sodium salt of alkylarylsulfonate) which is an excellent emulsifier and antistat due to its high ionization, about 5 weight percent of ethoxylated (20 ETO) tallow amine which is an excellent emulsifier and antistat, about 13 weight percent of ethoxylated 40 (4 ETO) lauryl alcohol emulsifier coupling agent, about 2 weight percent of sodium salt of nonyl sulfosuccinate which is an excellent wetting agent, and 2 weight percent of an antioxidant 4,4'-thio-bis-(6-tert butyl m1cresol).

The process finish composition is applied onto the yarn 45 in such a way as to allow about 0.3 to about 0.6 weight percent of said composition to be initially applied and with from about 0.15 to about 0.30 weight percent retained on the yarn to protect the fiber surface, required lubricity, and antistatic properties. During the heat treatment 50 of the yarn subsequent to the application of the process finish composition, about 40 to about 50 weight percent of the composition is volatilized. The volatiles consist mainly of the low viscosity mineral oil which contains a very low level of the other necessary components. The 55 volatiles are condensed and can be recovered through an exhaust system. The remaining process finish composition provides adequate surface lubrication, antistatic properties and antioxidant to protect the yarn surface during the subsequent drawing operation. An excellent advantage of this 60 process finish composition is that even when exposed to extremely high temperatures as required in a polyester spin draw or conventional spinning and drawing process, it suffers substantially no decomposition, thus preventing possible deposits on processing rolls and other threadpath components that affect processing efficiency.

The process finish composition is unique not only due to its composition which provides all requirements of lubrication, antistatic properties and protection from heat degradation, but because of its following physical properties which are essential or critical for uniformity of application and efficient fiber thermal treatment. First, low

viscosity of less than 40 centipoises at 25° C. by Brookfield Viscometer, for application at room temperature is critical. Second, good wetting ability measured by contact angle method on polyester film is necessary. A contact angle of less than 10° gives substantially ideal conditions of finish spreadability. Third, the eight component spin process finish composition is a uniform blend, water clear, and free of any suspended solids. In order to achieve this, an almost perfect HLB (hydrophylic-lipophylic balance) is achieved without adverse effects on any of the other essential properties of the finish composition. Just a minor variation or modification of ratio of the composition ingredients results in an unstable blend of cloudy appearance with suspended solids or complete separation of layers. Fourth, the composition yields low specific heat and the lowest possible heat of vaporization of the more volatile components which provides good conditions to minimize heat losses during the thermal treatment of the fiber. This limitation is one of the more critical limitations that aqueous compositions and emulsions cannot overcome as will be shown in the examples wherein process conditions as well as physical properties of the yarn cannot be obtained that are comparable to this invention. And, lastly, the composition is heat stable when exposed to high process temperatures and further, undergo substantially no chemical degradation even after partial volatilization or steam distillation.

The yarn finish or overfinish composition is applied onto the yarn in such a way as to allow about 0.7 to about 1.2 weight percent to remain on said yarn to improve its translational efficiency of yarn to tensitized cord, adhesion, heat stability, fatigue and tire durability properties. The yarn or overfinish composition can be applied

at any stage of the process subsequent to the critical drawing stage, thus yielding the unexpected possibilities of tailoring the surface properties of the fiber by additives for improving adhesion, thermal stability, fatigue, etc. Either one of two yarn finish compositions have been found to be adequate in accordance with this invention.

The improved yarn finish composition for use as the overfinish or yarn finish compositions in accordance with this invention consist of either (a) about 95 to about 98 weight percent of said composition of triethylene glycol-dipelargonate and about 2 to about 5 weight percent of said composition of 2,2-methylene-bis-(4-methyl-6-tertiary nonoylphenol) and (b) about 13 to about 25 weight percent of said composition selected from the group consisting of glycerol monoleate and decaglycerol tetraoleate with ethoxylated tall oil fatty acids, about 12 to about 20 weight percent of said composition selected from the group consisting of sulfated glycerol trioleate and ethoxylated alkylamine, and about 55 to about 75 weight percent of said composition of hexadecyl (isocetyl) stearate.

The yarns of this invention can be processed by any spin draw process or spinning and separately drawing process available to the art in the patent and technical literature, using any suitable polyester which provides the high tenacity yarn of about 9 grams per denier and minimum elongation of about 13 percent.

The following examples illustrate in Tables I, II, and III, applicant's present invention and advantages obtained thereby by interrelating finish compositions to fiber process performance and end product of yarn and cord physical properties. They are illustrative only and are not to be construed as limitative.

TABLE I—FINISH COMPOSITIONS

| Finish identities                                                               | Finish compositions, parts by weight |       |       |       |       |       |       |       |       |       |       |                      |
|---------------------------------------------------------------------------------|--------------------------------------|-------|-------|-------|-------|-------|-------|-------|-------|-------|-------|----------------------|
|                                                                                 | A                                    | B     | C     | D     | E     | F     | G     | H     | J     | K     | L     | Function             |
| <b>Finish components:</b>                                                       |                                      |       |       |       |       |       |       |       |       |       |       |                      |
| Refined coconut glyceride                                                       | 15.0                                 | 30.0  | 14.7  | 14.5  | 18.0  | 20.3  | ..... | 10.5  | ..... | ..... | ..... | Lubricant.           |
| Hexadecyl (isocetyl) stearate                                                   | 15.0                                 | ..... | 14.7  | 14.5  | 19.0  | ..... | 22.3  | 10.5  | ..... | ..... | ..... | Do.                  |
| Ethoxylated lauryl alcohol (4 EO)                                               | 13.0                                 | 13.0  | 12.7  | 12.7  | ..... | ..... | ..... | ..... | ..... | ..... | ..... | Emulsifier.          |
| Sodium petroleum sulfonate 60-62% active in mineral oil                         | 10.0                                 | 10.0  | 9.8   | 9.7   | ..... | ..... | ..... | ..... | ..... | ..... | ..... | Antistat emulsifier. |
| Ethoxylated tallow amine (20 EO)                                                | 5.0                                  | 5.0   | 4.9   | 4.9   | 10.0  | 1.4   | 1.4   | ..... | ..... | ..... | ..... | Do.                  |
| Sodium salt of sulfonated succinic ester                                        | 2.0                                  | 2.0   | 2.0   | 1.9   | ..... | ..... | ..... | ..... | ..... | ..... | ..... | Wetting agent.       |
| Sulfated glycerol trioleate                                                     | .....                                | ..... | ..... | ..... | 15.0  | 5.7   | 4.1   | 4.0   | ..... | ..... | ..... | Antistat emulsifier. |
| Ethoxylated tallow acid (1 EO)                                                  | .....                                | ..... | ..... | ..... | 2.8   | 2.7   | ..... | ..... | ..... | ..... | ..... | Emulsifier.          |
| Decaglycerol tetraoleate                                                        | .....                                | ..... | ..... | ..... | 2.1   | 1.7   | 0.7   | ..... | ..... | ..... | ..... | Do.                  |
| Glycerol monoleate                                                              | .....                                | ..... | ..... | ..... | 2.1   | 2.1   | ..... | ..... | ..... | ..... | ..... | Do.                  |
| Ethoxylated sorbitol oleate-laurate                                             | .....                                | ..... | ..... | ..... | ..... | ..... | 6.7   | ..... | ..... | ..... | ..... | Do.                  |
| Ethoxylated tallow glyceride                                                    | .....                                | ..... | ..... | ..... | ..... | ..... | 1.0   | ..... | ..... | ..... | ..... | Do.                  |
| Plastolein 9404 (triethylene glycol dipelargonate)                              | .....                                | ..... | ..... | ..... | ..... | ..... | 97.0  | ..... | ..... | ..... | ..... | Lubricant.           |
| Naugawhite (2,2-methylene-bis-(4-methyl-6-tert. nonyl-phenol))                  | .....                                | ..... | 3.0   | 3.0   | ..... | ..... | 3.0   | 3.0   | 3.0   | ..... | ..... | Antioxidant.         |
| Santowhite crystals (4,4 thio-bis(6-tert.-butyl-m-cresol))                      | 2.0                                  | ..... | ..... | 0.6   | 0.7   | 0.7   | ..... | ..... | ..... | ..... | ..... | Do.                  |
| Triethylene glycol di-short chain fatty acids (C <sub>5</sub> -C <sub>8</sub> ) | .....                                | ..... | ..... | ..... | ..... | 97.0  | ..... | ..... | ..... | ..... | ..... | Lubricant.           |
| Neopentyl glycol di-pelargonate                                                 | .....                                | ..... | 40.0  | 40.0  | 39.2  | 38.8  | 35.0  | ..... | ..... | 97.0  | ..... | Do.                  |
| Mineral oil viscosity 40 SSU                                                    | .....                                | ..... | ..... | ..... | 65.0  | 65.0  | 65.0  | 65.0  | 65.0  | ..... | ..... | Continuous phase.    |
| Water                                                                           | (1)                                  | (2)   | (1)   | (1)   | (2)   | (2)   | (3)   | (3)   | (3)   | (1)   | (1)   | (1)                  |
| Physical state at room temp.                                                    | .....                                | ..... | ..... | ..... | ..... | ..... | ..... | ..... | ..... | ..... | ..... | .....                |

<sup>1</sup> Clear oil blend. <sup>2</sup> Hazy oil blend. <sup>3</sup> Stable emulsion.

TABLE II.—FIBER PROCESS PERFORMANCE DATA

| Fiber finish identity                               | A    | B    | C    | C    | D    | E      | E     | F    | G    | H     | J        |
|-----------------------------------------------------|------|------|------|------|------|--------|-------|------|------|-------|----------|
|                                                     | (1)  | (2)  | (1)  | (1)  | (1)  | (2)    | (2)   | (3)  | (3)  | (3)   | (1)      |
| <b>Finish physical properties:</b>                  |      |      |      |      |      |        |       |      |      |       |          |
| Viscosity in centipoises (Brookfield)               | 22.5 | 25.0 | 29.0 | 29.0 | 26.0 | 26.0   | 26.0  | 7.8  | 11.0 | 9.2   | 15.6     |
| Contact angles on polyester in degrees              | 7.0  | 7.0  | 4.9  | 4.9  | 7.5  | 6.2    | 6.2   | 31.0 | 30.0 | 44.0  | 8.5      |
| Surface tension in dyn./cm.                         | 31.7 | 31.2 | 31.8 | 31.8 | 31.5 | 31.8   | 31.8  | 36.0 | 35.5 | 36.5  | 35.0     |
| <b>Manufacturing performance:</b>                   |      |      |      |      |      |        |       |      |      |       |          |
| Finish pick-up percent by wt. of fiber              | 0.45 | 0.45 | 0.45 | 2.20 | 0.45 | 0.45   | 1.50  | 1.65 | 3.10 | 2.90  | 1.55     |
| Finish oil on fiber by analysis, percent by wt.     | 0.2  | 0.2  | 0.2  | 1.2  | 0.2  | 0.2    | 0.8   | 0.5  | 0.7  | 0.8   | 0.7      |
| Drawing performance                                 | Exc. | Exc. | Exc. | Fair | Exc. | Good   | Fair  | Fair | Poor | Poor  | Very bad |
| Breaks and wraps/lb.                                | 0    | 0.01 | 0    | 0.09 | 0.01 | 0.04   | 0.09  | 0.07 | 0.13 | 0.18  | 0.25     |
| Deposits on draw heater                             | None | None | Neg. | Med. | Neg. | Slight | Heavy | Med. | Med. | Heavy | Heavy    |
| <b>Yarn properties:</b>                             |      |      |      |      |      |        |       |      |      |       |          |
| Ultimate tensile strength, g./d.                    | 8.5  | 8.5  | 8.6  | 8.5  | 8.4  | 8.6    | 8.5   | 8.6  | 8.5  | 8.5   | 8.3      |
| Ultimate elongation at break, percent               | 14.7 | 14.4 | 14.6 | 14.2 | 14.2 | 14.5   | 15.3  | 14.2 | 14.7 | 14.1  | 15.2     |
| Yarn quality rating <sup>4</sup> (broken filaments) | 2    | 2    | 1    | 1    | 1    | 2      | 2     | 3    | 4    | 4     | 5        |
| Yarn uniformity rating <sup>4</sup>                 | 1    | 1    | 1    | 3    | 1    | 1      | 3     | 4    | 5    | 5     | 4        |
| Sample number                                       | 1    | 2    | 3    | 4    | 5    | 6      | 7     | 8    | 9    | 10    | 11       |

<sup>1</sup> Clear oil. <sup>2</sup> Hazy oil. <sup>3</sup> Aqueous emulsion. <sup>4</sup> Rating: 1=best, 5=worst.

TABLE III.—YARN TIRE CORD PROPERTIES

| Fiber process finish identity.....                | C                | G                | A    | C    | A    | A     |
|---------------------------------------------------|------------------|------------------|------|------|------|-------|
| Yarn overfinish identity.....                     | ( <sup>1</sup> ) | ( <sup>1</sup> ) | G    | J    | K    | L     |
| Yarn sample identity.....                         | 12               | 13               | 14   | 15   | 16   | 17    |
| Total finish oil on yarn, percent by wt.....      | 0.2              | 0.7              | 1.2  | 1.3  | 1.3  | 0.9   |
| Yarn:                                             |                  |                  |      |      |      |       |
| Breaking strength in lbs.....                     | 24.9             | 24.4             | 24.5 | 24.5 | 24.6 | 25.0  |
| Percent elongation at break.....                  | 13.0             | 13.9             | 13.3 | 12.8 | 12.9 | 13.1  |
| Dipped tensilized cord:                           |                  |                  |      |      |      |       |
| Breaking strength in lbs.....                     | 61.7             | 62.4             | 64.2 | 65.2 | 66.3 | 63.9  |
| Percent elongation at break.....                  | 13.1             | 14.7             | 15.2 | 15.3 | 16.1 | 15.4  |
| Translational efficiency, percent.....            | 82.6             | 84.7             | 87.3 | 88.7 | 89.8 | 85.2  |
| Thermal stability, percent retained strength..... | 81.7             | 75.5             | 79.3 | 79   | 80.3 | 77.8  |
| Adhesion 3/8", hot.....                           | 32               | 33               | 32   | 36   | 33   | 30    |
| Adhesion 3/8", cold.....                          | 40               | 46               | 41   | 43   | 42   | 44    |
| Disk, fatigue, percent.....                       | 65.8             | 68.0             | 83.4 | 76.5 | 80.2 | 77.6  |
| Wheel life (hours).....                           | 79               | 60               | 104  | 98   | 84   | ----- |

<sup>1</sup> No finish.

I claim:

1. Synthetic filamentary yarn comprised of polyethylene terephthalate filaments which are first treated with 20 from about 0.3 to about 0.6 weight percent based on the weight of the yarn of a liquid composition consisting essentially of about 10 to about 20 weight percent of said composition of each hexadecyl stearate and refined coconut oil, about 3.0 to about 6.0 weight percent of 25 said composition of ethoxylated tallow amine, about 10 to about 20 weight percent of said composition of ethoxylated lauryl alcohol, about 8.0 to about 12.0 weight percent of said composition of sodium salt of alkylaryl-sulfonate about 1.0 to about 3.0 weight percent of 30 dinonyl-sodium-sulfosuccinate, about 1.0 to about 3.0 weight percent of said composition of 4,4' - thio-bis-(3-methyl - 6 - tert-butylphenol), about 35 to 50 weight per-

cent of said composition of white mineral oil having a boiling point of between 510° F. and 620° F. and a viscosity of between 38 to 40 SSU at 100° F. wherein at least about 0.15 to about 0.30 weight percent is retained on said yarn, and then said yarn is treated with from about 0.7 to about 1.2 weight percent on said yarn of a liquid composition selected from the group consisting of (a) about 95 to about 98 weight percent of said composition of triethylene glycol-dipelargonate and about 2 to about 5 weight percent of said composition of 2,2' - methylene - bis - (4 - methyl - 6 - tert. nonylphenol), and (b) about 13 to about 25 weight percent of said composition selected from the group consisting of glycerol monoleate and decaglycerol tetraoleate with ethoxylated tall oil fatty acids, about 12 to about 20 weight percent of said composition selected from the group consisting of sulfated glycerol trioleate and ethoxylated alkylamine, and about 55 to about 75 weight percent of said composition of hexadecyl (isocetyl) stearate.

## References Cited

## UNITED STATES PATENTS

|           |        |        |       |             |
|-----------|--------|--------|-------|-------------|
| 3,428,560 | 2/1969 | Olsen  | ----- | 117—139.5 X |
| 3,563,892 | 2/1971 | Cooley | ----- | 117—138.8 X |
| 3,575,856 | 4/1971 | Anton  | ----- | 117—138.8 X |

WILLIAM D. MARTIN, Primary Examiner

T. G. DAVIS, Assistant Examiner

U.S. Cl. X.R.

117—76 T, 139.5 CQ, 139.5 F; 252—8.75, 8.8, 8.9